

## UNITED STATES PATENT OFFICE

2,570,473

METHOD OF RECOVERING TIN FROM  
TIN-BEARING MATERIALS

Irving E. Muskat and Robert H. Taylor, Plainfield, N. J., assignors to The Vulcan Detinning Company, a corporation of New Jersey

No Drawing. Application May 17, 1946,  
Serial No. 670,547

3 Claims. (Cl. 23—136)

1

This invention is directed to the recovery of tin from tin ores and other tin-bearing materials by an improved process involving the sulfidizing of the tin content and the volatilization of the resulting tin sulfide, which can be collected and treated to recover the tin by known methods.

It is known to recover tin from tin-bearing materials such as tin ore by the conversion of the tin content of the material undergoing treatment to a sulfide and the subsequent volatilization of the resulting tin sulfide. It is also known that better yields of tin are obtained in accordance with such processes if the sulfidizing reaction is carried out in the presence of a reducing agent. In one such process the tin ore is heated to a reducing temperature below the fusion temperature and at that time there is brought in contact with the heated ore a liquid or solid reducing agent and a non-gaseous sulfidizing agent to effect the conversion and volatilization of tin sulfide. In another such process the tin ore is heated in the presence of a reducing agent and a sulfur compound to a temperature at which reduction occurs, and the heating of the mixture is continued until conversion of the tin and volatilization of the resulting tin sulfide is effected.

Insofar as we are aware, none of these prior art tin ore sulfidizing processes has met with commercial success because fusion of the ore took place with consequent substantial impairment of the yields of recoverable tin, at the sulfidizing and volatilization temperatures of about 950° C. to 1100° C. Moreover, the time required to effect sulfidization and volatilization of tin sulfide from the ore in accordance with these prior art processes was so inordinately long as to make their use commercially unfeasible.

We have found that if the tin ore is preliminarily reduced and if this reduction is carried out to an extent sufficient to make the reduced tin soluble in an aqueous alkali metal hydroxide solution at a temperature of at least about 75° C. to 90° C., that when this reduced ore is sulfidized at temperatures of about 950° C. to 1100° C. to volatilize the tin from the ore as tin sulfide no fusion or no substantial fusion of the ore takes place. In consequence there is a greater yield of recoverable tin than in the prior art processes referred to above. Additionally, these greater yields of recoverable tin are obtained in considerably less time than heretofore. For example, we have obtained approximately 95% of

2

the tin content of a Bolivian ore containing about 22% of tin in the form of tin sulfide by reacting this ore in a reduced state in accordance with our invention with sulfur at sulfidizing and volatilizing temperatures of about 1100° C., for approximately one-quarter to one-half hour. Similar yields were obtained at lower sulfidizing and volatilizing temperatures of about 1020° C. to 1060° C., in times varying from about one-half to one hour.

In carrying out the present invention with a tin ore as the starting material, the tin ore, either high grade or low grade and concentrated or unconcentrated, either with or without preliminary roasting to remove sulfur, is subjected to controlled reducing conditions so as to convert the tin content of the ore into a state in which most if not all of the tin is soluble in an aqueous alkali metal hydroxide solution, at a temperature in the order of at least about 75° C. to 90° C. and up to the boiling point of the solution. By soluble it is meant that the tin is in a form in which it may be converted to a water soluble stannate by reaction with an aqueous alkali metal hydroxide, of a concentration of about 15% and, of course, higher, preferably in the presence of an oxidizing agent capable of oxidizing metallic tin in an alkaline medium, at the aforesaid temperature. For substantially all tin ores, including the low grade tin ores of 5 to 35% tin content, the reduction is sufficiently complete in accordance with the present invention if the tin content is soluble in an aqueous alkali metal hydroxide solution which contains 130 gms. NaOH and 40 gms. NaNO<sub>3</sub> per liter of solution, at a temperature of about 90° C. Equivalent amounts of other alkali metal hydroxides may be used in the solution as may also equivalent amounts of other oxidizing agents capable of oxidizing metallic tin in an alkaline medium, such as potassium nitrate, sodium hypochlorite, hydrogen peroxide, etc.

After the ore has been reduced to the aforesaid state it is reacted with a sulfur-containing material at temperatures sufficiently high to effect sulfidization of the reduced tin and volatilization of the resulting tin sulfide. The sulfidizing reaction may be carried out in any suitable vessel such as a direct-fired rotary kiln, for example, either in a neutral atmosphere or a reducing atmosphere, preferably the latter. Oxidizing atmospheres should be avoided because such atmospheres induce oxidization of the tin and other metals in the ore and thereby cut down

the yields of recoverable tin and add to the cost of the process.

Where the tin content of the reduced ore is high, say in the order of about 35-40% and higher, it is preferred to effect the sulfidization of the reduced ore in the presence of a solid carbonaceous reducing agent, such as coal in a powdered state, in substantially uniform admixture with the reduced ore. This added solid carbonaceous reducing agent is a safeguard against fusion of the reduced ores at the sulfidizing and volatilizing temperatures of up to about 1100° C. The amount of solid carbonaceous reducing agent which may be added to the reduced ore to prevent fusion may vary rather widely, as desired, from about 5% to 40%, based on the weight of the ore.

Any sulfur-containing material, solid, liquid or gas, capable of reacting with tin at a temperature of from about 950° C. to 1100° C. to form a tin sulfide may be used in accordance with the present invention. The amount of sulfidizing agent which may be used may vary widely, from about 10% to 100% or even more, based on the weight of the tin-containing material being treated, in the case of sulfur. Equivalent amounts of other sulfur-containing materials such as ferrous sulfide, sulfur dioxide, sulfur-containing petroleum crudes, etc., may be used. Sulfur, however, is preferred because more of the tin is sulfidized and in less time than with the other sulfidizing agents. Optimum results are usually obtained with a low grade reduced tin ore containing from about 15 to 35% of tin by using from about 25% to 50% of sulfur, based on the weight of the ore.

The temperature at which the reduced tin ore is sulfidized and the tin volatilized therefrom in the form of a tin sulfide may vary from about 950° C. to 1100° C., the preferred temperatures varying from about 1020° C. to 1100° C. The time of treatment of the ore with a sulfidizing agent at these temperatures may vary widely, from about 15 minutes upwardly. Usually the maximum amount of tin is volatilized in the form of tin sulfide in about 15 minutes to one-half hour, although at times it is essential to prolong the reaction to about one hour in order to volatilize the maximum amount of tin out of the ore, particularly at lower sulfidizing and volatilizing temperatures in the order of about 950° C. to 1050° C. Generally, sulfidizing reaction times in excess of about one hour are ineffective to increase to any substantial extent the amount of tin which can be volatilized from the ore in the form of tin sulfide in accordance with our process.

In the practice of the process herein contemplated to effect reduction, a tin ore in a finely divided state is heated in the presence of a quantity of a solid carbonaceous reducing agent capable of reducing tin oxide to metallic tin, such as carbon, coal, lampblack, petroleum coke, etc. for a time required and at a predetermined temperature to convert the tin content of the ore into the aforesaid soluble state. The ore treated may contain from about 5% to 60% and even more of tin, including both high grade and low grade ores, although for economic reasons it is preferred to treat a low grade tin concentrated or unconcentrated ore containing from about 15% to 35% or less of tin.

The reduction treatment of the ore is effected by heating the ore in a pulverized state, for example, minus 100 or 200 mesh, in the presence

of a solid carbonaceous reducing agent such as coal, charcoal, carbon and coke, preferably in powdered form and preferably of a mesh corresponding substantially to the mesh of the ore. These solid carbonaceous reducing agents are preferred because they are easier to handle and because they have the property of minimizing fusion and sintering of the ore. Solid carbonaceous materials containing both nonvolatile and volatile carbonaceous reducing agents, such as anthracite or bituminous coal, are most suitable for this purpose. Bituminous coal is preferred because of its relative cheapness and availability.

The reduction treatment should be conducted at a temperature sufficiently high to permit a major part or all of the tin content of the ore to be converted to the aforesaid aqueous alkali soluble state; however, the temperature should not be so high that substantial fusion occurs and a molten pool of ore, slag or metallic tin or other molten material is formed. A ball mill or other suitable grinding device may be employed to grind the ore to the desired finely divided state. The ore may be ground to minus 20 or 60 mesh, but better yields of reactable tin are obtained if the ore is ball-milled to the mesh above stated.

The exact temperature which may be utilized in the reducing treatment is dependent largely upon the nature of the ore subjected to reduction. Thus, some Bolivian ores fuse or melt to a very serious extent at a temperature of about 870° C. On the other hand, other Bolivian ores and many Mexican ores may be subjected to temperatures as high as about 980° C. or 1040° C. without encountering serious fusion. Slight amounts of fusion resulting in some sintering of the ore undergoing treatment may be tolerated in most cases. On the other hand, fusion to an extent such that pools of molten material are formed is detrimental and should be avoided. In general, satisfactory results are usually obtained within a temperature range of about 760° C. or 815° C. to about 1100° C. and for most tin ores a temperature of from about 870° C. to 1040° C. is most effective. A preferred temperature range is from about 900° C. to 1000° C.

The period of time over which the ore is subjected to the reducing treatment is capable of considerable variation, being largely dependent upon the activity of the ore undergoing treatment and the temperature of treatment. Generally speaking, the time required is shorter where the temperature is high than where a lower temperature is used. In any case, however, unduly prolonged heat treatment of the ore is detrimental and should be avoided. The actual optimum time at the reduction temperature is usually quite short and usually does not exceed about 30 to 40 minutes for low-grade ores. From data obtained by carrying out experiments in a reduction furnace, it appears that low-grade ores may be reduced to a good product in a matter of from about 8 to 12 minutes and even less. These figures include the time required to heat the ore up to the reduction temperature, which in typical instances was shown to be in the order of about 3 to 5 minutes. The reduction may be effected in any suitable furnace, such as a hearth type furnace, for example, a multiple hearth, Wedge type furnace, or a rotary furnace.

The amount of reducing agent utilized is, in general, dependent upon the temperature of treatment and the type of furnace in which reduction is effected. It has been observed that

fusion of the ore may be substantially decreased and minimized when the process is conducted in the presence of an excess of solid carbonaceous material such as carbon or coal. In treatment of ores, particularly low grade ores containing from about 15 to 35 per cent of tin, not less than about two times the amount of carbon or coal required to reduce tin to the metallic state and form carbon monoxide is preferred. When this reduction is conducted in a continuous manner by use of a rotary kiln or a multiple hearth furnace or other similar device, not less than about 15 to 20 per cent by weight of carbon or coal, based upon the weight of the ore, is used for most cases, since with these amounts of solid carbonaceous material the tendency of the ore to fuse and sinter at the temperature of reduction is greatly lessened. In general, coal in excess of about 30 per cent by weight is undesirable where the temperature is unduly high or the treatment unduly long because coking may occur. The minimum or theoretical amount of bituminous coal, for example, required for reduction of the tin in a typical low-grade Bolivian ore of about 20% to 22% tin content is about 5% of the weight of the ore.

Following the reducing treatment the ore is, preferably, cooled in a nonoxidizing atmosphere to prevent reoxidation of the tin. The cooled reduced ore is thereafter sulfidized. This cooling treatment is not essential for the heated reduced ore may be treated with a sulfidizing agent, particularly a sulfidizing agent in a gaseous state, normal or otherwise, in accordance with the present invention.

The reduced ore after the cooling treatment usually is in the form of a black or dark colored pulverulent or granular mass containing tin in dispersed small particles in a form soluble in the aforesaid aqueous alkali solutions. Sometimes the mass may be more or less clinkered or caked and may require a pulverizing or grinding treatment, say to minus 100 or 200 mesh, prior to the sulfidizing treatment at temperatures of from about 950° C. to 1100° C. In the preferred operation, the reduced ore prior to the sulfidizing treatment should be in a finely divided state such as set forth above.

The exact nature of the reducing reactions is not known, although it is possible that the tin is reduced to a finely divided metallic state, the particles being separated by the excess coal and by other materials in the reduced ore. In any event, this reduced ore is more amenable to reaction with a sulfidizing agent, particularly sulfur, than is ore not similarly treated.

The following example is illustrative of a preferred embodiment of the present invention.

The ore preparatory to the sulfidizing treatment was roasted and reduced as follows:

Ore containing about 21% tin, 22% iron, 19% silica, 2% sulfur, and other impurities in minor amounts was roasted in an oil-fired rotary furnace in an oxidizing atmosphere at a temperature of about 815° C. The roasted ore, which contained about 0.7% sulfur, was ball-milled to a particle size passing a 100-mesh screen. 100 parts by weight of the milled ore was intimately mixed with 20 parts of powdered bituminous coal. The mixture was fed into an oil-fired rotary furnace maintained at a maximum temperature of about 980° C. and operated with a reducing atmosphere. The ore-coal mixture was fed in at a rate such that it passed through the furnace in about 15 minutes. The reduced ore was cooled

in a non-oxidizing atmosphere and then ball-milled to pass a 100-mesh screen.

Approximately 20 parts by weight of the reduced ball-milled ore were intimately mixed with 10 parts by weight of powdered sulfur and the mixture was placed in a vessel and the latter was heated for 30 minutes at a temperature of 1100° C., in a non-oxidizing atmosphere of nitrogen. Under these conditions approximately 95% of the tin content of the ore was volatilized in the form of tin sulfide.

In a similar experiment with the same reduced tin ore-sulfur charge at a temperature of 1060° C. for 30 minutes, approximately 94% of the tin content was volatilized from the ore. In another similar experiment with the same reduced tin ore, using 20 parts by weight of the ore, 5 parts by weight of powdered sulfur and a temperature of 1060° C. for one hour, approximately 95% of the tin content was volatilized from the ore.

It is manifest that the details as to time and temperature of reduction of the tin ore and time and temperature of sulfidization of the reduced ore may be varied, as may also the proportions of coal to ore in the reduction treatment and sulfur to reduced ore in the sulfidizing treatment, all as hereinabove set forth. It is also manifest that other sulfidizing agents such as ferrous sulfide, etc. may be used, although not with the especially desirable results obtained with sulfur.

Although the invention has particular value for the treatment of tin ores, including tin ore concentrates and naturally occurring minerals containing tin, it may also be applied to the recovery of tin from other tin-containing materials such as tin-containing dressing plant tailings or the spent tin ore residues from other tin recovery processes. Thus, for example, it may be applied to the spent residues from the aqueous alkali leaching process of recovering tin from reduced tin ores which is described and claimed in the co-pending application to one of us, Serial No. 614,825, filed September 6, 1945, now Patent No. 2,416,709.

In accordance with the process of the application to one of us, tin ore is reduced to such an extent that the tin content is soluble in an aqueous alkali metal hydroxide solution as herein described. The reduced tin ore is then treated with an aqueous alkali metal hydroxide to form an alkali metal stannate which is leached from the ore. The residues from that process are the spent residues hereinabove referred to. These spent residues are tin-containing materials in a reduced state in accordance with the present invention. They contain varying amounts of tin, from about 1% to 8%.

These spent residues may be mixed with a sulfidizing agent with additional reduction and sulfidized in accordance with the present invention, either with or without the presence of a solid carbonaceous reducing agent. Thus, for example, when 20 parts of a ball-milled spent residue containing 2.4% tin from the alkali process of the aforesaid application were mixed with 10 parts of powdered sulfur and sulfidized at 1060° C. for 30 minutes as herein described, approximately 87% of the tin content was volatilized in the form of tin sulfide. With the same spent residue and 12 parts of powdered sulfur and 4 parts of powdered coal, using again a temperature of 1060° C. for 30 minutes, approximately 90% of the tin content was volatilized in the form of tin sulfide.

The recovery of the tin from the tin sulfide forms no part of our invention. Any of the con-

ventional methods may be used for this purpose, such as those referred to in the British Patent No. 361,402, accepted November 18, 1931, for example.

In our copending application Serial No. 670,548, filed on even date herewith, there is disclosed and claimed a process of recovering tin in the form of tin sulfide from a tin-containing ore, in which process a uniform mixture of an unreduced low grade tin ore, an excess of a solid carbonaceous reducing agent and a sulfidizing agent is heated in a non-oxidizing atmosphere at a temperature of about 950° to 1100° C., for a time sufficient to volatilize the resulting tin sulfide from the ore undergoing treatment.

We claim:

1. A process for recovering tin in the form of tin sulfide from a low grade tin ore containing about 15% to 35% of tin in a form in which it is in a substantially aqueous alkali-insoluble state, comprising heating such ore in the presence of about 5% to 40% of a solid carbonaceous reducing agent, based on the weight of the ore, at a temperature of at least about 760° C. but below that at which the ore fuses, under conditions such that reduced ore containing tin in dispersed small particles in a form soluble in aqueous alkali solution at a temperature of at least about 75° C. to 90° C. is produced, and heating the product of such treatment containing the said soluble tin with a sulfidizing agent at a temperature of about 950° C. to 1100° C. to form tin sulfide and for a time sufficient to volatilize the same from the ore undergoing treatment.

2. A process for recovering tin in the form of tin sulfide from a low grade tin ore containing about 15% to 35% of tin in a form in which it is in a substantially aqueous alkali-insoluble state, comprising heating such ore in the presence of about 5% to 40% of a solid carbonaceous reducing agent, based on the weight of the ore, at a temperature of at least about 760° C. but below that at which the ore fuses, under conditions such that reduced ore containing tin in dispersed small

particles in a form soluble in aqueous alkali solution at a temperature of at least about 75° C. to 90° C. is produced, and heating the product of such treatment containing the said soluble tin with about 25% to 50% by weight of sulfur at a temperature sufficiently high to form tin sulfide and for a time sufficient to volatilize the same from the ore undergoing treatment but below that at which the ore fuses.

3. A process for recovering tin in the form of tin sulfide from a low grade tin ore containing about 15% to 35% of tin in a form in which it is in a substantially aqueous alkali-insoluble state, comprising heating such ore in the presence of about 5% to 40% of a solid carbonaceous reducing agent, based on the weight of the ore, at a temperature of at least about 760° C. but below that at which the ore fuses, under conditions such that reduced ore containing tin in dispersed small particles in a form soluble in aqueous alkali solution at a temperature of at least about 75° C. to 90° C. is produced, and heating the product of such treatment containing the said soluble tin with a sulfidizing agent at a temperature sufficiently high to form tin sulfide and for a time sufficient to volatilize the same from the ore undergoing treatment but below that at which the ore fuses.

IRVING E. MUSKAT.  
ROBERT H. TAYLOR.

#### REFERENCES CITED

The following references are of record in the file of this patent:

UNITED STATES PATENTS

| Number    | Name          | Date         |
|-----------|---------------|--------------|
| 1,606,343 | Burdick       | Nov. 9, 1926 |
| 1,847,991 | Sulman et al. | Mar. 1, 1932 |

FOREIGN PATENTS

| Number  | Country       | Date          |
|---------|---------------|---------------|
| 316,177 | Great Britain | Nov. 27, 1930 |